

# UNITED STATES PATENT OFFICE.

CHARLES S. DOLLEY, OF PHILADELPHIA, PENNSYLVANIA.

## PROCESS OF TANNING.

SPECIFICATION forming part of Letters Patent No. 630,494, dated August 8, 1899.

Application filed October 21, 1896. Serial No. 609,600. (No specimens.)

*To all whom it may concern:*

Be it known that I, CHARLES S. DOLLEY, a citizen of the United States, residing at Philadelphia, in the county of Philadelphia and State of Pennsylvania, have invented certain new and useful Improvements in Processes of Tanning; and I do declare the following to be a full, clear, and exact description of the invention, such as will enable others skilled in the art to which it appertains to make and use the same.

This invention relates to improvements in tanning hides or skins; and the objects of the invention are to provide a single-step tanning process which is simple, inexpensive, efficient, and rapid, and to produce a soft, tough, and pliable leather sound in texture and which is free from discoloration and harmful foreign matters and is well adapted to be finished and colored by any of the ordinary finishing and coloring methods and agents.

My invention consists, essentially, in subjecting the hide or skin to be tanned to the action of formic aldehyd ( $\text{CH}_2\text{O}$ ) in such manner and proportion and for such time that the hide or skin under treatment shall be thoroughly permeated by the formic aldehyd, which I have discovered will under proper conditions form an insoluble compound with the gelatinous constituents of the hide or skin and at the same time effect those other chemical and physical changes essential to the conversion of a raw hide or skin into leather.

In carrying out my process I take a hide or skin which has been prepared for tanning by one of the commonly-employed modes, according to the particular character of the hide or skin under treatment, and I subject said prepared hide or skin to the action of formic aldehyd either in its natural gaseous condition or in aqueous solution, the degree of concentration of the gas or the strength of the solution and the time of treatment varying, of course, with the character and thickness of the hide or skin to be tanned.

If the formic aldehyd be employed in the form of an aqueous solution, I have found the following an advantageous method to pursue for the conversion of ordinary goat-skins into Morocco leather: I begin the treatment with preferably, say, a three-per-cent. solution of

the formic aldehyd and treat the skins in this solution in a closed drum for, say, ten minutes, adding formic aldehyd to the solution 55 at intervals of, say, ten minutes until at the end of an hour, or thereabout, the solution has been brought up to a strength of ten per cent. and the hides have thus in the interval been subjected to the continuous action of 60 a tannage solution of gradually-increasing strength. I have found in practice that ordinary goat-skins treated as above described may be thoroughly tanned in a period of an hour, or thereabout.

The hides or skins should be subjected to the ordinary tests known to tanners from time to time during the process and should be allowed to remain and to be agitated or re- 70 volved in the drum until said tests applied to the thickest portions of the thickest hides or skins under treatment indicate to a person skilled in the art thorough permeation and through and through conversion of the hide into leather, the hide or skin having lost the 75 triply translucent appearance and peculiar feel of a raw hide and become opaque and colorless and leathery to the touch through and through.

If the formic aldehyd be used in a gaseous state, I suspend the hides or skins to be tanned in a chamber capable of being hermetically closed and connected with any suitable form of apparatus for generating formic-aldehyd gas. The skins being suspended within this 85 chamber and the door closed, the formic-aldehyd gas is introduced into the chamber, and this is continued and the hides or skins subjected to the action of the gases or mixed 90 gas and vapor, until the ordinary tests indicate to a person skilled in the art that the hides or skins have been thoroughly permeated by the tanning agent and that the conversion of the hide or skin into leather is complete.

If the formic aldehyd be employed in a gaseous state, I find that as many ordinary prepared goat-skins in a moist condition as can be suspended in a tight chamber having a capacity of, say, two thousand cubic feet may 100 be thoroughly tanned within a period of from six to ten hours by the action of the quantity of formic-aldehyd gas generated by the ordinary process from one liter of wood-alcohol.

The formic aldehyd may also be employed in the gaseous state by the vaporization of an aqueous or alcoholic solution, and I find that if it be used in this manner it is desirable to add a proportion of chlorid of calcium to the formic-aldehyd solution, polymerization of the formic aldehyd being in this manner largely prevented. For this purpose two hundred parts of chlorid of calcium for each fifteen hundred parts of formic-aldehyd solution suffices. In case the gas is employed in connection with aqueous vapor it should of course be understood that live or heated steam is not employed, but rather a cool vapor or moisture-charged atmosphere.

It sometimes occurs that a batch of skins which by reason of their unusual thickness or from other cause may require a strength of the tanning solution differing somewhat from that employed in tanning ordinary hides or skins, and it is at once evident that in such case the tanner may readily, by selecting a fair specimen of the batch of skins to be tanned and using the same as a test for the strength of the tannage solution required, more readily determine the strength of the solution which may be required in tanning such hides or skins.

I understand leather, technically speaking, to be the peculiar product resulting from the action of a tanning agent upon the collagen and connective tissue constituents of animal hide or skin, which product is characterized and distinguished from raw skin by chemical peculiarities varying with the special tanning agent employed in all cases, by the fact that the tanning agent has entered into a fixed combination with the skin substances and is not to be recovered, as are the salt and alum used in tawing; also, by the fact that certain physical alterations are produced—such, for example, as being insoluble and non-putrescible—and by a difference in density, elasticity, and permeability to light and water familiar to persons skilled in tanning. Leathers produced by different agents have different chemical characters, though possessing a general physical resemblance. Thus the "tano-gelatin," which, according to certain authorities, (Watt, page 314,) is produced by the use of tannic acid, being a different substance from the chromatized gelatin of the chrome process. My leather is made from skin or hide by producing a chemical combination be-

tween formic aldehyd and the collagen and connective tissue of animal skin, and as a new article of manufacture is to be distinguished from other leathers—such as oak, hemlock, or chrome leather—by any or all of the following tests: first, by coming from the tanning-bath free from any discoloration due to the tanning agent; second, by its freedom from material deposits—such as the pigment, ross, resin, &c., deposited in the skin in bark-tannage—or from the product of the reduction of mineral salts, as in mineral tannage, and, third, by any or all of the various tests for formic aldehyd, inasmuch as a certain amount of this substance when used as a tanning agent remains in an uncombined state in the skin, in which it may be detected.

Having thus described my invention, what I claim to be new, and desire to secure by Letters Patent, is—

1. As a new article of manufacture, a tanned hide or skin, consisting essentially of a combination of formic aldehyd with the collagen and other gelatinous constituents of the said hide or skin, substantially as herein set forth. 75
2. As a new article of manufacture, leather obtained by treating animal hide or skin with formic aldehyd, thereby rendering insoluble and non-putrescible the collagen or connective tissue substances of the skin, such leather consisting essentially of a combination of 85 formic aldehyd with the collagen and other gelatinous constituents of the said hide or skin, substantially as set forth.
3. The herein-described process of tanning, that is to say, subjecting the hide or skin to 90 be tanned to the action of formic aldehyd,  $(CH_2O_2)$  substantially as herein set forth.
4. The process herein described of tanning, that is to say, subjecting the hide or skin to be tanned, to the action of formic aldehyd, 95  $(CH_2O_2)$  commingled with aqueous vapor, substantially as herein set forth.
5. The process of tanning, which consists in subjecting the hide or skin to be tanned, to the action of formic aldehyd,  $(CH_2O_2)$  employed in solution, substantially as set forth. 100

In testimony whereof I affix my signature in presence of two witnesses.

CHARLES S. DOLLEY.

Witnesses:

CHAS. O. MORTON,  
H. F. REARDON.